

## UNITED STATES PATENT OFFICE

2,665,443

## ASTATIC BRUSH FOR GROOMING THE HAIR

Simon A. Simon, Longmeadow, and Arthur H. Drelich, Springfield, Mass., assignors, by mesne assignments, to Chicopee Manufacturing Corporation, Chicopee Falls, Mass., a corporation of Massachusetts

No Drawing. Application June 4, 1949,  
Serial No. 97,302

4 Claims. (Cl. 15—159)

1

Dielectric materials, particularly plastics, generate electrostatic charges when rubbed with various other dielectric materials, including hair, clothing, fur, etc. This causes the hair to stand out or separate when it is groomed with a comb or brush made of such plastics, and even produces uncomfortable shocks. Generation of static is reduced or eliminated by dipping the hairbrush or comb in a dilute dispersion of particular chemical substances (identified herein) and then drying.

It has long been known that various materials which are classed non-conductors of electricity and called dielectrics have the inherent property of generating static charges of electricity when rubbed with various other dielectric materials. Such electrostatic generating materials are extremely numerous. They include wool, fur, hair, bristles, dried varnish, and most of the members of that large class of materials popularly known as plastics. It is common knowledge that articles made of these materials in everyday use develop electrostatic charges, probably as a result of unavoidable friction, and that these electrostatic charges have many undesirable results which include the production of uncomfortable shocks and dangerous sparks, standing out of hair upon brushing, and extraordinary attraction and retention of dust.

As used herein, the term astatic denotes absence of the property or ability to generate, induce or accumulate objectionable electrostatic charges, and the term antistatic pertains to reducing or eliminating the property or ability to generate, induce or accumulate electrostatic charges. That is, an antistatic agent tends to produce an astatic result.

As used herein, the term plastic has a meaning more restricted than the indefinite sense in which it is popularly used. As used herein, plastic designates a non-cellulosic high polymer (usually but not necessarily organic) of synthetic origin (as opposed to being found in nature) and either molded into a solid or capable of being so molded. This definition includes, for example, saran and other vinyl resins; methacrylate resins; polystyrene; polyethylene; nylon; polytetra-fluoro-ethylene and others.

Instruments for grooming the hair including hair-brushes and combs normally are made of or contain dielectric materials such as plastics and bristles. Bristles may be either natural hog bristles or filaments of nylon or other plastic. Rubbing these materials against the hair generates objectionable electrostatic charges.

2

It has been proposed to render various material astatic by coating with antistatic agents or possibly chemically combining antistatic agents with dielectric materials. However, in the instances which have come to our attention, the proposed treatments have not been completely successful for one or a number of reasons. For example, some materials such as saran and polytetra-fluoro-ethylene are so smooth and so chemically inert that it has been regarded as impossible to cause any materials either to combine with them or adhere to them. Some proposed antistatic coatings for other materials so change the properties of the material or its surface as to make it undesirable for other reasons, although it might have astatic properties. Also, although materials are known which for a time impart some degree of astatic character to some dielectrics, such astatic properties are not sufficiently lasting to be satisfactory, for example, either because the antistatic materials readily wash off or are otherwise removed in normal use, or because the astatic property rapidly diminishes and disappears. Other proposed antistatic agents are hygroscopic and undesirably attract water to the surfaces to which they are applied, and this prevents their being useful in many instances.

We have discovered that the materials in a certain group or class, which we designate by the coined word etymols, have antistatic properties, and that they combine with various dielectric materials (not necessarily in the chemical sense) or adhere to such dielectrics, particularly those plastics which are the subject of this invention, and when so combined or adhered render the dielectrics astatic.

The etymols are defined as long chain fatty acid partial esters (including the poly-oxy-alkylene ethers of such esters) of the following:

- A. those aliphatic poly-hydroxy alcohols having from two to six carbon atoms and from two to six hydroxyl groups;
- B. monomeric cyclic ethers of such poly-hydroxy alcohols;
- C. polymeric ethers having at least two hydroxyl groups and which may be considered condensation products of such poly-hydroxy alcohols.

The etymols include, for example, the following materials arranged as sub-groups of A, B, and C above:

- a. glyceryl esters such as glyceryl monostearate, mono-oleate, etc. and poly-oxy-ethylene propylene glycol mono-stearate

- b. long chain fatty acid partial esters of the hexitans (that is esters of monomeric cyclic ethers of hexitol) and hydroxy-poly-alkylene ethers thereof such as sorbitan mono-laurate, and sorbitan mono-laurate poly-oxy-ethylene ether.
- c. polyethylene glycol esters, such as polyethylene glycol mono-stearate, mono-oletate, etc., and the polyethylene-glycol ether of poly-propylene-glycol mono-stearate.

We have discovered that the etymols are particularly effective in imparting astatic properties to plastics, that the etymols surprisingly combine with or adhere to various inert and smooth or slippery plastics (for example saran and polyethylene) and together with such materials form astatic articles or substances. We have also discovered that certain of these etymols, although readily dispersible in water, nevertheless when placed upon certain plastics impart a durable astatic character thereto, which resists scrubbing and washing.

Based on these discoveries, it is an object of our invention to render astatic normally electrostatic plastics and thus to provide materials with desirable mechanical and physical properties for many uses for which they were formerly unsuitable because of undesirable electrostatic properties.

Also based on these discoveries it is an object of our invention to provide an improved instrument for grooming the hair which will not generate electrostatic charges in use.

Our invention can be applied to hairbrushes, combs and the like of any known or suitable construction where such brushes and combs include dielectric material, such as natural bristles, nylon bristles, saran bristles, methacrylate resin backs, etc. In carrying out our invention, we dip, brush or spray the instrument with a dilute dispersion or solution of a suitable etymol in a volatile carrier such as water, alcohol, or carbon tetrachloride and then dry. We prefer the water dispersion. We have found surprisingly that the etymols adhere to, combine with (not necessarily in the chemical sense) or otherwise cooperate even with inert plastics such as saran to provide a durable astatic combination. This combination resists both dry abrasion (incident to use) and with some etymols, repeated scrubbing with a stiff bristle brush and water or soap solution (incident to cleaning). These results and these properties are contrary to what is to be expected from the individual properties of the plastic and the etymols. Thus saran is known for its very smooth surface and high degree of chemical inertness. Consequently heretofore it has been considered impossible to combine anything with saran or to make anything adhere to it. Also while many of the etymols are regarded as insoluble in water, they are readily dispersible. Consequently it is contrary to the known properties both of the plastics and the etymols that they form a combination and that this combination resists separation by active scrubbing.

Moreover very small quantities of the etymols produce an astatic combination with the plastics, even with saran. We have found that a concentration of  $\frac{1}{8}\%$  of sorbitan mono-laurate, for example, in the treating dispersion produces a noticeable astatic effect, and that the saran can be rendered completely astatic by concentrations of less than 1%. The tabulation below shows the range of concentrations of a water disper-

sion of sorbitan mono-laurate which we have found effective to render the saran astatic. A closely woven fabric of saran monofilaments was dipped in dispersions of the concentrations indicated, and after drying was rubbed briskly with a woolen cloth. The saran was then brought near a sensitive electroscope.

In the tabulation below the numerical values of needle deflection are approximately proportional to the voltage induced on a very sensitive deflecting needle electroscope. The deflection 5 represents the highest induced voltage which we have found to be permissible. That is a piece of saran cloth, charged to a voltage of 5 as shown by this electroscope, will discharge so as to produce a noticeable shock to a person connected with it. A deflection of greater than 5 indicates that the shock will be uncomfortable and objectionable. A deflection of less than 5 will not produce noticeable or objectionable shock.

|    | Percent Concentration of Antistatic Dispersion | Needle Deflection |
|----|------------------------------------------------|-------------------|
| 25 | $\frac{1}{64}$                                 | 10                |
|    | $\frac{1}{32}$                                 | 9                 |
|    | $\frac{1}{16}$                                 | 7                 |
|    | $\frac{1}{8}$                                  | 5                 |
|    | $\frac{1}{4}$                                  | 2                 |
|    | $\frac{1}{2}$                                  | 0                 |
| 30 |                                                | 0                 |

As will be seen from the tabulation a dispersion of  $\frac{1}{8}\%$  markedly reduces the charge that can be induced on the plastic, and may be said to represent the minimum operative concentration of the particular etymol sorbitan mono-laurate when used with saran, while a concentration of  $\frac{1}{4}\%$  reduces the charge to a value well within the acceptable range and  $\frac{1}{2}\%$  eliminates static completely.

We do not know the exact nature of the resulting plastic treated with the etymols. Apparently evaporation of the carrier from dispersions of low concentration does not leave a simple film or coating which can be identified and described as such. And as yet we have no positive evidence that there is any chemical combination between the plastic and etymol. The only way we can define the treated combination of plastic and an etymol is to say that this combination has electrostatic properties substantially identical with the plastic which has been covered with a dispersion of the etymol.

As indicated by the tabulation, concentrations of sorbitan mono-laurate greater than  $\frac{1}{2}\%$  satisfactorily eliminate static, but we have found that concentrations above about 2% give the saran fabric an objectionable feel. Therefore, we use concentrations within the range  $\frac{1}{8}\%$  to 2% and prefer to use between  $\frac{1}{4}\%$  and 1%.

#### Example I

A hairbrush having a methacrylate resin back and nylon bristles when used to brush the hair, dry, and under given conditions causes the hair to stand out objectionably. The brush is dipped in a  $\frac{1}{4}\%$  dispersion in water of sorbitan mono-laurate and dried. Thereafter brushing the same hair under the same conditions produces no observable static and no objectionable standing out.

#### Example II

A hairbrush having a lacquered wood back and natural bristles when used to brush the hair, dry, and under given conditions causes the hair to stand out objectionably. The brush is dipped

in a  $\frac{1}{4}\%$  dispersion in water of sorbitan mono-laurate and dried. Thereafter brushing the same hair under the same conditions produces no observable static and no objectionable standing out.

The class of etymols includes a large number of substances which are closely related in chemical structure and antistatic properties. For example, the aliphatic poly-hydroxy alcohols from which the partial esters and ethers thereof can be derived include ethylene glycol; di- and tri-ethylene glycol; glycerol and polyglycerols, pentaerythritol; pentitols; hexitols and the monomeric cyclic ethers thereof; cyclitols such as inositol; oligosaccharides such as glucose, sucrose and lactose; the glycol and lower polyglycol ethers of the above named poly-hydroxy alcohols. The esters of the mixed monomeric cyclic ethers of the hexitols (such as sorbitans and sorbides, mannitans and mannides) and the poly-oxy-alkylene ethers thereof are suitable etymols. The hydroxy-poly-oxy-ethylene ethers of these esters can be prepared by reacting the partial ester with a preformed polyethylene glycol or with 10 to 30 mols of ethylene oxide. Such reaction products are known in the literature and are named, for example, "reaction products of sorbitan mono-laurate with 20 mols ethylene oxide," or more simply "sorbitan mono-laurate poly-oxy-ethylene ether." Specific etymols which we have found suitable antistatics are:

Diethylene glycol mono-laurate  
 Diethylene glycol mono-stearate  
 Ethylene glycol mono-laurate  
 Ethylene glycol mono-myristate  
 Ethylene glycol mono-ricinoleate  
 Glyceryl mono-laurate  
 Glyceryl mono-myristate  
 Glyceryl mono-oleate  
 Glyceryl mono-ricinoleate  
 Mannitan di-laurate poly-oxy-ethylene ether  
 Mannitan mono-oleate  
 Mannitan mono-oleate poly-oxy-ethylene ether  
 Mono-penta-erythritol ester of soy oil fatty acids  
 Penta-erythritol mono-oleate  
 Penta-erythritol mono-stearate  
 Polyethylene glycol mono-laurate  
 Polyethylene glycol mono-myristate  
 Polyethylene glycol mono-oleate  
 Polyethylene glycol mono-ricinoleate  
 Polyethylene glycol mono-stearate  
 Poly-oxy-ethylene propylene glycol mono-stearate  
 Propylene glycol mono-myristate  
 Propylene glycol mono-oleate  
 Propylene glycol mono-stearate  
 Propylene glycol mono-ricinoleate  
 Sorbitan mono-laurate  
 Sorbitan mono-laurate poly-oxy-ethylene ether  
 Sorbitan mono-naphthenate  
 Sorbitan mono-oleate  
 Sorbitan mono-oleate poly-oxy-ethylene ether  
 Sorbitan mono-palmitate  
 Sorbitan mono-palmitate poly-oxy-ethylene ether  
 Sorbitan mono-stearate  
 Sorbitan mono-stearate poly-oxy-ethylene ether  
 Sorbitan tri-oleate  
 Sorbitan tri-oleate poly-oxy-ethylene ether

While the etymols generally impart astatic qualities to the plastics, there are measurable differences in the intensity and durability under various conditions of these qualities which have been effected by the various specific etymols.

For example, the degree of reduction of static for a given concentration of applied dispersion varies from etymol to etymol. Thus the concentration of the etymol dispersion originally applied varies. Also a large number of etymols originally impart a satisfactory or equal degree of astatic property to the plastic, but there are variations in the life of the astatic property in use (resistance to friction) and in the resistance of the astatic property to cleaning or scrubbing. There is also a variation from etymol to etymol of the astatic properties of the plastic at low temperature such as 20° F.

However, the nature, extent and durability of the astatic property achieved by any specific etymol appears to be independent of the plastic to which the etymol is applied, at least as far as can be detected in ordinary conditions of use. Thus sorbitan mono-laurate applied at a given concentration of dispersion for example, appears to impart substantially equal astatic properties to saran, polyethylene, various vinyl resins, methacrylate resins, nylon, poly-tetra-fluoro-ethylene, etc.

Of the etymols named, we prefer glyceryl mono-oleate because of its ready availability and easy application, and because it gives satisfactory astatic properties even at low temperatures which have long shelf life and are resistant to friction, and to washing. Other particularly effective etymols are poly-oxy-ethylene propylene glycol mono-stearate, glyceryl mono-ricinoleate, polyethylene glycol mono-oleate, sorbitan mono-laurate, sorbitan mono-stearate poly-oxy-ethylene ether and sorbitan tri-oleate and poly-oxy-ethylene ether, pentaerythritol mono-oleate.

Also, we may use blends or mixtures of the etymols to combine the good properties of several. Thus we may combine for example, an etymol giving particularly good astatic properties at low temperature with one having exceptional resistance to washing to obtain an antistatic agent having both properties.

It will be understood that our invention is not limited to the illustrations of the foregoing explanation, but includes what is defined within the scope of the appended claims.

We claim as our invention:

1. A hair brush comprising in combination plastic bristles which have been covered with a dilute dispersion of a compound selected from the group consisting of long chain fatty acid partial esters and poly-oxy-alkylene ethers of long chain fatty acid partial esters of a compound selected from the group consisting of aliphatic poly-hydroxy alcohols having from two to six carbon atoms and from two to six hydroxyl groups, monomeric cyclic ethers of aliphatic poly-hydroxy alcohols having from two to six carbon atoms and from two to six hydroxyl groups, and polymeric ethers having at least two hydroxyl groups which are condensation products of aliphatic poly-hydroxy alcohols having from two to six carbon atoms and from two to six hydroxyl groups in a volatile carrier and dried.

2. A hair brush comprising in combination natural bristles which have been covered with a dilute dispersion of a compound selected from the group consisting of long chain fatty acid partial esters and poly-oxy-alkylene ethers of long chain fatty acid partial esters of a compound selected from the group consisting of aliphatic poly-hydroxy alcohols having from two to six carbon atoms and from two to six hydroxyl groups, monomeric cyclic ethers of aliphatic

poly-hydroxy alcohols having from two to six carbon atoms and from two to six hydroxyl groups, and polymeric ethers having at least two hydroxyl groups which are condensation products of aliphatic poly-hydroxy alcohols having from two to six carbon atoms and from two to six hydroxyl groups in a volatile carrier and dried.

3. A hair brush comprising in combination a plastic normally dielectric back and bristles protruding from the back, said brush having been covered with a dilute dispersion of a compound selected from the group consisting of long chain fatty acid partial esters and poly-oxy-alkylene ethers of long chain fatty acid partial esters of a compound selected from the group consisting of aliphatic poly-hydroxy alcohols having from two to six carbon atoms and from two to six hydroxyl groups, monomeric cyclic ethers of aliphatic poly-hydroxy alcohols having from two to six carbon atoms and from two to six hydroxyl groups, and polymeric ethers having at least two hydroxyl groups which are condensation products of aliphatic poly-hydroxy alcohols having from two to six carbon atoms and from two to six hydroxyl groups in a volatile carrier and dried.

4. A hair brush comprising in combination a plastic normally dielectric back and bristles protruding from the back, said brush having been dried after being covered with dispersion of a compound selected from the group consisting of long chain fatty acid partial esters and poly-oxy-alkylene ethers of long chain fatty acid partial esters of a compound selected from the group

consisting of aliphatic poly-hydroxy alcohols having from two to six carbon atoms and from two to six hydroxyl groups, monomeric cyclic ethers of aliphatic poly-hydroxy alcohols having from two to six carbon atoms and from two to six hydroxyl groups, and polymeric ethers having at least two hydroxyl groups which are condensation products of aliphatic poly-hydroxy alcohols having from two to six carbon atoms and from two to six hydroxyl groups in a volatile carrier containing between about  $\frac{1}{8}\%$  and about 1% of the said compound.

SIMON A. SIMON.  
ARTHUR H. DRELICH.

15 References Cited in the file of this patent

UNITED STATES PATENTS

| Number    | Name        | Date           |
|-----------|-------------|----------------|
| 2,041,213 | Schellenger | May 19, 1936   |
| 2,266,561 | Marick      | Dec. 16, 1941  |
| 2,287,766 | Davis       | June 30, 1942  |
| 2,290,880 | Katzman     | July 28, 1942  |
| 2,297,135 | Davis       | Sept. 29, 1942 |
| 2,311,818 | Dawson      | Feb. 23, 1943  |
| 2,359,750 | Collins     | Oct. 10, 1944  |
| 2,390,437 | Hayes       | Dec. 4, 1945   |
| 2,393,863 | Myers       | Jan. 29, 1946  |
| 2,397,471 | Cox         | Apr. 2, 1946   |
| 2,418,752 | Brown       | Apr. 8, 1947   |
| 2,426,315 | Marick      | Aug. 26, 1947  |
| 2,441,945 | Frolich     | May 25, 1948   |
| 2,461,043 | Eisen       | Feb. 8, 1949   |